

## UNITED STATES PATENT OFFICE

2,658,000

SOLUTION FOR TREATMENT OF FIBROUS  
CELLULOSIC MATERIALS

William F. Sullivan, Roseland, and Irene M. Panik, Elizabeth, N. J., assignors to National Lead Company, New York, N. Y., a corporation of New Jersey

No Drawing. Application May 31, 1951,  
Serial No. 229,272

5 Claims. (Cl. 106—15)

1

This invention relates to treated cellulosic material, and is a continuation-in-part of our co-pending application Serial No. 134,342, filed December 21, 1949, now abandoned. More specifically it relates to fire resistant material. Still more specifically it relates to flame resistant, cellulosic materials and a method for their production.

Many types of agents have been proposed for rendering cloth, paper and other fibrous materials fire resistant, and some have been successfully employed, but few have the necessary properties to be able to withstand the rigors of handling and cleaning, particularly of washing and laundering. Some of the known treating agents are capable of being washed and laundered to a limited degree, but most of them appreciably alter the appearance, texture or tensile strength of the treated cellulosic material. In addition many of the known agents are not sufficiently adherent and tend to separate from the treated material in the form of fine dust.

Among the fire retarding agents which are non-launderable are the phosphate, borate and sulfamate types. Launderable types of agent include resins, chlorinated resins, or waxes added in combination with inorganic oxides such as antimony oxide. They, however, have the disadvantage of altering the appearance of the material considerably, and that they must be added in large quantity. Titanium has been added in several fire resistant processes, but in most of these the titanium has been added as titanium dioxide in order to obtain opaque pigment effects.

An object of this invention is, therefore, to provide an agent useful in the treating of fibrous cellulosic materials to render the same fire resistant. Another object is to provide an agent for the treatment of fibrous cellulosic materials to impart flame- and glow-resistant properties thereto which will not be affected by washing or laundering. A still further object is to provide a solution for the treatment of fibrous cellulosic materials to render the same fire resistant, which will not alter the appearance, texture or tensile strength of the material. A further object is to produce fire resistant fibrous cellulosic materials in which the appearance, texture and tensile strength of the materials have not been altered by the treating agent. These and other objects of the present invention will become apparent as the invention is more fully described.

In its broadest aspects this invention contemplates production of a fire resistant or non-inflammable fibrous cellulosic material by im-

2

pregnating the material with an aqueous solution of titanium chloride acylate which is capable of forming a transparent gel, gelatinizing said solution on said material to form a transparent gel, alkalizing said gel-containing material with an alkaline neutralizing agent and subsequently washing and drying said material. For improved flame resistance together with resistance to afterglow, the above process may be carried out using an aqueous solution of titanium chloride acylate which contains antimony chloride, and this improved process is also contemplated by this invention. This invention further contemplates fibrous cellulosic materials which have been rendered flame resistant by the present process.

A titanium salt solution useful in the practice of this invention for treatment of fibrous cellulosic material to impart fire resistance thereto comprises an aqueous solution of titanium chloride acylate. The solution may also contain antimony chloride for improved and superior results. The titanium chloride acylates are derivatives of orthotitanic acid,  $Ti(OH)_4$ , in which some of the hydroxyl groups of the orthotitanic acid have been replaced by chloride ions, and others have been replaced by acylate groups. An acylate group, as used here, is understood to mean a derivative of a carboxylic acid obtained by removal of the carboxyl hydrogen of the acid.

It has been found that satisfactory results are obtained when the titanium concentration in the aqueous solution of titanium chloride acylate is between 40 and 150 grams per liter, preferably about 60 grams per liter, the concentration of chloride may be from 0.75 to 2.25 parts for each part of the titanium, and the concentration of acylate from 1.25 to 3.70 parts for each part of titanium. When antimony chloride is used the concentration of antimony may be from 1.0 to 3.0 parts for each part of titanium, and an additional amount of chloride should be present to form antimony trichloride. The chloride values in the antimony chloride are in addition to the chloride values of the titanium chloride acylate.

Among the fibrous cellulosic materials which may be rendered fire resistant by the process of the instant invention are fabrics such as cotton, linen, regenerated cellulose, viscose and cellulose acetate, also natural fibers such as kapok, hemp, wood and wood products such as pressed boards, cardboard, batting, paper, wood flour, sawdust, and the like. The cellulosic material is treated with the titanium salt solution by any convenient means, such as by dipping the material in

the solution, or by spraying the solution on the material. Any excess solution on the cellulosic material may be removed, for example, by squeezing between rolls, deliquoring in a filter press, or any other appropriate method depending upon the physical nature of the material. It is preferred to leave a quantity of solution on the material about equal to the weight of the material itself, i. e. a weight pick-up of about 100%. The titanium salt solution impregnated in the cellulosic material is gelatinized, for example by exposing the treated material to the atmosphere for a short interval of time. Satisfactory results have been obtained when the exposure is such as to reduce the weight of solution held by the cellulosic material to about  $\frac{1}{2}$  to  $\frac{1}{4}$  of its original weight. The cellulosic material containing the gelatinized treating agent is then subjected to an alkalizing agent in order to raise the pH of the treated material to, above 7.5, preferably above 9.0, but not exceeding about 12.0. The type of alkalizing agent used is unimportant although weak alkalizing agents such as, for example, sodium carbonate or ammonium hydroxide or carbonate, are preferred. The material is then rinsed well with water, for example by decantation, in order to remove the soluble salts therefrom and subsequently dried.

It has been found that the preferred amount of impregnant on the final material (dry basis) is about 6.0% to 9.0% of the weight of the fibrous cellulosic material when the titanium chloride acylate solution is used alone, while about 14% to 16% is preferred when the combination of titanium chloride acylate and antimony chloride is employed.

The entire process may be carried out at room temperature although, if desired, temperatures up to 60° C. may be employed.

The exact nature of the physical and chemical changes that take place during this process is not completely understood. However, the solution of titanium chloride acylate is apparently converted to a transparent gel which adheres tenaciously to the cellulosic material and is not removed by subsequent washing. It may be held in the pores or between the fibers of the cellulosic material, may be absorbed or adsorbed on the surface or may react to some extent with the cellulosic material itself.

To illustrate preferred embodiments of this invention, the following examples are presented:

#### EXAMPLE I

In order to prepare an aqueous solution of titanium chloride acetate the following procedure was used:

Two parts of lead acetate ( $Pb(C_2H_3O_2)_2 \cdot 3H_2O$ ) were dissolved in one part of water by weight at 65° C. The lead acetate solution was added slowly to a solution of titanium tetrachloride, containing 180 grams per liter titanium. The amount of lead acetate solution used was equivalent to react with 65% of the chloride values present in the titanium tetrachloride solution. The time of addition of the lead acetate solution to the titanium tetrachloride was 2 hours in order to maintain the temperature of the mixture below 25° C. The mixture was then filtered to remove the lead chloride from the titanium chloride acetate solution.

The titanium chloride acetate solution contained 77 grams per liter of titanium, 262 grams per liter of acetate, and 70 grams per liter chloride.

The titanium chloride acetate solution was diluted with water to produce a solution containing 60 grams per liter titanium. This solution was used for treating cloth. The cloth was cotton twill weighing 8.2 ounces per square yard.

The cloth was immersed in the solution for 2½ minutes and was passed through a hand wringer. The operation was repeated the second time (immersed and wrung again) to obtain good soaking. The treated cloth was then partially dried by exposing the cloth to the atmosphere for 2 hours to gelatinize the treating agent on the cloth. The gelatinized treated cloth was then immersed for 5 minutes in a solution of sodium hydroxide containing 200 g. p. 1 NaOH to alkalinize the solution retained on the cloth. The pH of the retained solution held by the cloth was 9.5. The excess solution was squeezed out of the cloth by passing the cloth through a hand wringer. The cloth was then washed well with water until the retained solution had a pH of 8.0. The washed cloth was then thoroughly dried. The entire procedure was carried out at room temperature. The treated cloth was subjected to the standard flame test and the results are recorded in Table I.

The standard flame test is called the 45° microburner test and consists of exposing the smooth side of the fabric at an angle of 45°  $\frac{3}{4}$  inch above the top of a burner. The flame,  $1\frac{1}{4}$  inches in length, is played on to the fabric for 12 seconds. The afterflaming and afterglow data are recorded in seconds. The procedure and apparatus assembly has been developed by the Quartermaster Corps of the United States Army and is described by Robert W. Little, Major in Quartermaster Corps, in his book entitled "Flameproofing Textile Fabrics" on pages 117-119, Reinhold Publishing Corporation, 1947.

#### EXAMPLE II

To form an aqueous solution containing the combination of titanium chloride acetate and antimony chloride, another portion of the titanium chloride acetate solution used in Example I was taken and admixed with antimony chloride solution to form a treating solution containing 60 grams per liter titanium and 68.3 grams per liter antimony.

The cloth was treated in the same manner as described in Example I except the drying temperature was 50° C. and the drying time was 15 minutes and ammonium hydroxide solution was added as an alkalizing agent instead of sodium hydroxide. The treated cloth was subjected to the standard flame test and the results are recorded in Table I.

Table I

|                                    | Example I           | Example II                              |
|------------------------------------|---------------------|-----------------------------------------|
| Treating solution used             | Ti-chloride acetate | Ti-chloride acetate + antimony chloride |
| Afterflame (sec.)                  | 0                   | 0                                       |
| Afterglow in uncharred area (sec.) | >60                 | 0                                       |
| Charred area (sq. in.)             | 4.5                 | 4.5                                     |
| Tensile strength                   | Fair                | Good                                    |
| Hand                               | Good                | Do.                                     |
| Appearance                         | do                  | do                                      |

From Table I it is clearly shown that flame resistant properties have been imparted to the cloth treated with a solution of titanium chloride acetate when used alone or in combination with antimony chloride; and when used

in combination with the antimony chloride the cloth also exhibits glow resistant properties.

EXAMPLE III

A third portion of the titanium chloride acetate solution used in Example I was diluted to 60 grams per liter titanium and used for treating wood flour.

The wood flour was immersed in the solution and agitated for 10 minutes to insure thorough soaking. The excess solution was separated from the wood flour by deliquoring on a filter press. The filter cake was then removed from the press and partially dried by 3 hours' exposure to the atmosphere to gelatinize the solution on the wood flour. This treated, partially-dried wood flour was then immersed in a solution of 150 grams per liter  $\text{Na}_2\text{CO}_3$  and agitated for 10 minutes to alkalize the solution on the wood flour, and again deliquored. The pH of the retained solution in the wood flour was 9.8. The wood flour was then thoroughly washed in water until the pH of the retained solution was 7.8 and dried. The treated wood flour was tested for flame retardation by holding in the flame of a Bunsen burner for several seconds. It was observed to char only and did not flame. Untreated wood flour when tested similarly flamed immediately and was almost entirely consumed.

While the examples shown illustrate employment of titanium chloride acetate solution, which is preferred, solutions of titanium chloride formate and titanium chloride propionate may be used with similar effect. These compounds, however, are somewhat more expensive to produce and therefore not as economical as the acetate salt.

By means of the present invention it also has been found that fibrous cellulosic material treated with the titanium chloride acylate solution retains flame resistance after laundering. The laundering is carried out in a tumbling chamber with 0.5% neutral soap solution at 70° C. However, when the preferred method of this invention is employed, utilizing the combination of titanium and antimony compounds as described, the superior flame and glow resistance characteristics are retained even after repeated laundering. After 6 launderings, for instance, the results are identical to those before laundering.

These results are compared in Table II with a well-known treating agent which consists of a mixture of borax, boric acid, and diammonium hydrogen phosphate.

Table II

|                                                           | After laundering | After-flame (sec.) | After-glow in uncharred area (sec.) | Charred area (sq. in.) |
|-----------------------------------------------------------|------------------|--------------------|-------------------------------------|------------------------|
| Ti-chloride-acetate.....                                  | 1 time.....      | 25                 | >60                                 | 10.4                   |
| Ti-chloride-acetate+anti-mony chloride.....               | do.....          | 0                  | 0                                   | 4.5                    |
| Ti-chloride-acetate+anti-mony chloride.....               | 6 times.....     | 0                  | 0                                   | 4.5                    |
| Borax, boric acid, and diammonium hydrogen phosphate..... | 1 time.....      | (1)                | (1)                                 | (1)                    |

<sup>1</sup> Completely burned.

A fibrous cellulosic material treated with a solution of titanium chloride acetate retains a

useful measure of flame resistant properties upon laundering. However, when the cellulosic material is treated with the combination of agents, that of a solution of titanium chloride acetate and antimony chloride, the flame and glow resistant characteristics are maintained after repeated laundering. The combination of agents apparently produces a synergistic effect which enhances the flame resistance as well as imparting glow resistance and results in retention of these characteristics after laundering. The agents employed are fixed by employment of the process of this invention and are rendered durable toward washing.

Recoveries of both titanium and antimony values are substantially 100 per cent during processing. The amounts of titanium and antimony originally absorbed on the fibrous cellulosic material are equal to the amounts retained in the final material after processing.

When the titanium values are present in the material in substantially opaque form, the treated material has an unpleasant white tone and a white dust may be continually removed from the surface. By the utilization of the process of this invention, however, the titanium values are fixed in the material in a form in which substantially no alteration in appearance or texture of the material is observed. The treatment process is simple, convenient and economical to use. By employment of this invention, fibrous cellulosic materials may be treated to render them permanently resistant to fire.

While this invention has been described and illustrated by the examples shown, it is not intended to be strictly limited thereto and other modifications and variations may be employed within the scope of the following claims.

We claim:

1. A solution for treatment of fibrous cellulosic materials to impart fire resistance thereto comprising an aqueous solution of titanium chloride acylate, said acylate selected from the group consisting of formate, acetate and propionate, the titanium of said titanium chloride acylate being present in concentration from 40 to 150 grams per liter, the acylate group of said titanium chloride acylate being present in amount from 1.25 to 3.70 parts for each part of titanium present, the chloride of said titanium chloride acylate being present from 0.75 to 2.25 parts for each part of titanium present.

2. A solution according to claim 1 in which said acylate is acetate.

3. Solution according to claim 1 in which said acylate is formate.

4. Solution according to claim 1 in which said acylate is propionate.

5. A solution for treatment of fibrous cellulosic material to impart fire resistance thereto comprising an aqueous solution of titanium chloride acylate and antimony trichloride, said acylate selected from a group consisting of formate, acetate and propionate, the titanium of said titanium chloride acylate being present in concentration of 40 to 150 grams per liter, the acylate group of said titanium chloride acylate being present in amount from 1.25 to 3.70 parts for each part of titanium, the antimony of said antimony trichloride being present in amount from 1.9 to 5.75 parts for each part of titanium, the chloride of said titanium chloride acylate being present in amount from 0.75 to 2.25 parts

for each part of titanium in addition to the chloride present as antimony trichloride.  
 WILLIAM F. SULLIVAN  
 IRENE M. PANIK.

References Cited in the file of this patent  
 UNITED STATES PATENTS

| Number    | Name           | Date         |
|-----------|----------------|--------------|
| 2,547,671 | Sastmax et al. | Apr. 3, 1951 |
| 2,570,566 | Lane et al.    | Oct. 9, 1951 |

## FOREIGN PATENTS

| Number  | Country       | Date          |
|---------|---------------|---------------|
| 578,888 | Great Britain | July 16, 1946 |

## OTHER REFERENCES

Giua et al: Chem. Ab., vol. 19, page 1671<sup>6</sup>.  
 Helv. Chim. Acta., vol. 7, 1924, page 1082.  
 Giua et al.: Zeit. Anorg. Chem., vol. 166 (1927),  
 pp. 306-310.